

Sept. 12, 1933.

L. P. MELLERIO

1,926,161

SHOE STIFFENER AND METHOD OF MANUFACTURING THE SAME

Filed June 29, 1931

2 Sheets-Sheet 1

Fig.1.



Fig.2.



Fig.3.



INVENTOR  
Lucien P. Mellerio  
By his Attorney  
Harlow M. Davis

Sept. 12, 1933.

L. P. MELLERIO

1,926,161

SHOE STIFFENER AND METHOD OF MANUFACTURING THE SAME

Filed June 29, 1931

2 Sheets-Sheet 2

Fig. 4.



Fig. 5.



INVENTOR

Lucien P. Mellerio  
By his Attorney,  
Harlow M. Davis

## UNITED STATES PATENT OFFICE

1,926,161

SHOE STIFFENER AND METHOD OF  
MANUFACTURING THE SAME

Lucien Paul Mellerio, Leicester, England, assignor to United Shoe Machinery Corporation, Paterson, N. J., a corporation of New Jersey

Application June 29, 1931, Serial No. 547,565, and  
in Great Britain July 10, 1930

20 Claims.

(Cl. 36—77)

This invention relates to shoe stiffeners having a porous base which carries a stiffening substance and to methods of manufacturing them, and will be described, by way of illustration, as embodied in a toe stiffener of the so-called "semi-soft" type and with especial reference to the manufacture of such stiffeners.

In stiffeners of this type it is desirable to provide a greater amount of stiffening substance per unit volume in that portion which, in the finished shoe, will extend around the sides and end of the toe portion of the shoe and for a certain distance up from the junction of the upper with the sole, and to provide a less amount per unit volume in that portion of the stiffener which is uppermost in the finished shoe. The toe portion of the shoe will thus be very stiff and hard around the sides and end but will be quite flexible and resilient on the top. It is also desirable that a considerable portion at least of a toe stiffener, whether or not it is of this general type in which certain portions are more flexible than others, should be sufficiently pervious to permit diffusion of air and moisture outwardly from the inside of the shoe during wear; and the present invention provides a method whereby either or both of these desirable results may be attained.

In one aspect the method of this invention comprises subjecting a stiffener blank having a porous base, which carries a stiffening substance, to pressure to expel stiffening substance from a selected locality and to transfer it to another locality. In the case of a semi-soft stiffener a blank carrying a uniformly distributed load of stiffening substance, such for example as a mixture of colophony and Montan wax which is thermoplastic, may advantageously be subjected to heat and pressure by means of suitably formed rollers to expel some of the substance from the middle portion of the blank and to transfer it to a generally crescent-shaped locality lying along but spaced from the front and side edges thereof. There may thus be produced from an ordinary thermoplastic stiffener which was originally of a uniform stiffness throughout a semi-soft stiffener.

In another aspect the invention comprises a method of rendering a stiffener, or a selected locality of a stiffener, pervious to air and moisture. This locality may be the middle locality of a semi-soft stiffener of the type referred to above; and this result may be produced by suitably controlling the conditions of heat and pressure. To this end, a heat of suitable temperature to reduce the stiffening substance to a proper consistence is preferably employed, and a pressure of a force and duration is used just sufficient to expel a certain amount of stiffening substance without permanently consolidating the fabric base. Thus, after the pressure has been withdrawn and before

the stiffener has cooled, the fibres of the fabric will spring back to or toward their original positions so that pores or cracks will be formed in the comparatively small amount per unit volume of stiffening substance which remains after the expelling operation.

The invention also comprises a novel stiffener which may result from the practice of the method, and which, as herein illustrated, is characterized by having a porous base impregnated with a stiffening substance which is impervious to air and moisture, the stiffening substance in a part of the stiffener spaced from the margin of the stiffener, being sufficiently discontinuous to be pervious.

Referring now to the accompanying drawings, Fig. 1 is a plan of a toe stiffener made in accordance with the method of the invention;

Fig. 2 is a section on the line II—II of Fig. 1;

Fig. 3 is a section on the line III—III of Fig. 1;

Fig. 4 is a plan of a modified form of toe stiffener; and

Fig. 5 is a section on the line V—V of Fig. 4.

For producing a semi-soft toe stiffener, a suitably shaped blank may be cut to outline from the cold, hard impregnated sheet in the usual way. Assuming that the stiffener is for use in a man's shoe, and has a length of say 3½ inches on the line II—II and a width of say 4½ inches on the line III—III of Fig. 1, it may conveniently be cut from sheet fabric composed of porous sheet material of say 65 to 70 thousandths of an inch in thickness before impregnation, impregnated with the usual type of thermoplastic stiffening substance and calendered to be in the cold hard condition of a fairly uniform thickness of say 90 to 100 thousandths of an inch and to contain some 75% by weight of stiffening substance.

The blank thus prepared may then be subjected to heat and pressure by any suitable apparatus. For example, the apparatus shown in United States Letters Patent No. 1,704,818, granted March 12, 1929, upon an application filed in the names of William H. Bancroft, William J. Lund, and Maurice G. Hill, may be employed, with a suitably shaped die in the die roller and with the rolling pressure and the temperature so controlled that the following results are obtained. There is expelled from the entire margin enough stiffening substance so that a comparatively thin beveled margin results. Expulsion of stiffening substance is also caused to occur to a considerable extent from all portions of the blank except from a crescent-shaped locality indicated in Fig. 1 by a dot-and-dash line. In this locality the blank actually is left so heavily charged with stiffening substance that on both its faces, though to differing extents, there is (see a, b, Figs. 2 and 3) a crescent-shaped surface deposit of excess substance. As better illustrat-

ing the form of the die used in such a case during the hot-pressure treatment, the following particulars may be given regarding the thickness of one such treated blank when it has become cold 5 and stiff.

|    |  | Thickness of an inch                         |
|----|--|----------------------------------------------|
|    |  | Thickness at points <i>c</i> Fig. 1—about 30 |
| 10 |  | Thickness at points <i>d</i> Fig. 1—about 35 |
|    |  | Thickness at points <i>e</i> Fig. 1—about 40 |
|    |  | Thickness at points <i>f</i> Fig. 1—about 45 |
|    |  | Thickness at point <i>g</i> Fig. 1—about 50  |
| 15 |  | Thickness at points <i>h</i> Fig. 1—about 60 |
|    |  | Thickness at points <i>k</i> Fig. 1—about 70 |
|    |  | Thickness at points <i>l</i> Fig. 1—about 90 |

Such a cold stiff blank will have the usual marginal thinness of a skived blank; but, over the whole area embraced by the horns of the crescent-shaped locality, it will be tough and flexible having none of that hard, unyielding and somewhat brittle character which is a common attribute of the main portion of thermoplastic blanks as hitherto made. Moreover, over most of said tough and flexible locality the blank will be so porous as relatively freely to admit of the flow of air through it from one face to the other. This latter result is apparently due to the expulsion, without such excessive pressure as permanently to consolidate the cloth itself to an undue degree, of a sufficiency of stiffening substance to prevent the interstices of the fabric remaining filled with the substance when, after the pressure is relieved, the blank expands before it chills and sets hard. These stated characteristics of 35 toughness and flexibility of the stiffener, within the locality indicated, are apparently more or less completely retained in the stiffener in the finished shoe in spite of the heating to which the stiffener is subjected for the lasting operations and of the 40 tensions and pressures to which the softened stiffener is exposed during these operations which inevitably to some extent displace the softened stiffening substance. Such displacement appears, however, to result principally in an absorption of stiffening substance from the heavily charged crescent-shaped locality by the upper materials in immediate contact therewith and a 45 consequent disappearance of any perceptible undue thickness of the stiffener at that part. In 50 the finished shoe, the stiffened toe is very stiff and hard around the sides and end of the toe for a certain distance up from the junction of the upper and sole, the outer marginal portion of the stiffener between its outer edge and said 55 crescent-shaped locality furnishing the part of the stiffener which is lasted over upon the shoe bottom. The stiffener, however, is quite pliable and leathery on the top of the toe portion of the shoe. Conveniently, to ensure the correct location 60 of the said crescent-shaped locality of the stiffener with reference to the shoe upper during the lasting operations the stiffener and upper are fused together preparatory to the pulling-over operation by the employment of a suitable heated 65 press of usual construction. In such case it may be preferred to facilitate such union of stiffener and upper without depending upon any considerable heating or pressing of the stiffener in the press except at portions of the stiffener which 70 will be on the shoe bottom in the finished shoe; and this can be provided for by so forming the hot-rolling-die aforesaid that, adjacent to each corner of the stiffener indicated at *d* in Fig. 1, a spot of excess stiffening substance is left on 75 the blank, these spots being located respectively

in the two angles included between the rear edge and the side edges of the stiffener.

In some instances, when the toe stiffener is attached to the upper only by its corners as just been described, it may happen that, after 80 the shoe has been completed and subjected to wear, there will be a tendency for the rear margin of the stiffener between the ends thereof to part company from the adjacent portion of the upper so that wrinkles are produced across 85 the toe portion of the upper. In order to avoid this possibility the hot rolling-die, by which the stiffener is first subjected to heat and pressure, may be so formed that a thickened band of 90 stiffening substance may be caused to extend across the stiffener close to the rear edge of the stiffener, the outline of such a band being indicated by the dotted lines 7 and 9 in Fig. 4. In 95 this figure the thickness at the points indicated by the references *c*, *e*, *f*, *g*, *h*, *k* and *l* may be substantially the same as at the points indicated by the same references with regard to Fig. 1. This band or locality will preferably, as shown, be narrower at the mid line (V—V) of the stiffener and also of somewhat lesser thickness than 100 the main crescent-shaped locality, the thickness at the point *g* in the locality being about the same as that of the point *g* previously indicated. While such a narrow locality as last described 105 will in most instances secure due adhesion of the stiffener in the shoe and at the same time avoid giving undesired stiffness across the top of the toe when the stiffener is fused into an upper, it is contemplated that, where circumstances may require a greater assurance against 110 undue stiffening by such material which is furnished purely for securing adhesion, separated areas or spots positioned substantially along the line of the band may be used to secure the adhesion required instead of a continuous band. 115

Although the invention has been described in connection with the manufacture of a toe stiffener comprising a porous base impregnated with thermoplastic material, it should be understood that the invention is not limited in the scope of 120 its application to such stiffener or to such material.

Having thus described the invention, what I 125 claim as new and desire to secure by Letters Patent of the United States is:

1. The method of making shoe stiffeners which comprises subjecting a stiffener blank impregnated with a stiffening substance to pressure to cause the stiffening substance to be expelled from one locality of the blank and to be transferred to and deposited permanently in another locality of the blank. 130

2. The method of making a shoe stiffener which comprises subjecting a suitably shaped blank of porous sheet material impregnated with a stiffening substance to pressure in such manner as to expel stiffening substance from the middle portion of the blank and to deposit permanently the expelled stiffening substance in a locality the outer edge of which is spaced from 135 an edge of the blank. 140

3. The method of making a shoe stiffener which comprises subjecting a suitably shaped blank of porous sheet material impregnated with a stiffening substance to pressure in such manner as to expel stiffening substance from middle and marginal portions of the blank and to deposit permanently the expelled stiffening substance in a locality an outer edge of which lies 145 along but is spaced from an edge of the blank. 150

4. The method of making a shoe stiffener which comprises subjecting a suitably shaped blank of porous material impregnated with a stiffening substance to rolling pressure in such a manner as to expel stiffening substance from one locality and deposit it permanently in another locality of the blank. 80
5. The method of making a shoe stiffener which comprises preparing a suitably shaped blank of porous sheet material impregnated with a thermoplastic substance and subjecting the blank to heat and pressure in such manner as to expel thermoplastic substance from the marginal and middle portions of the blank and to deposit said expelled thermoplastic substance permanently in a comparatively narrow locality lying substantially parallel to that edge of the blank which is to be bent over upon the bottom of the shoe during the lasting operation. 85
- 10 6. The method of making a toe stiffener which comprises preparing a suitably shaped blank of porous sheet material impregnated with a thermoplastic substance and subjecting the blank to heat and pressure in such manner as to expel thermoplastic substance from the marginal and middle portions of the blank and to deposit said expelled thermoplastic substance permanently in a curved locality lying substantially parallel to the front and side edges of the blank. 90
- 15 7. The method of making shoe stiffeners which comprises subjecting a selected locality of a suitably shaped blank of porous sheet material impregnated with a thermoplastic stiffening which renders said material substantially impervious to air and moisture to pressure in such manner as to expel sufficient substance from said locality to render that locality pervious to air and moisture, and to transfer the expelled substance permanently to another locality. 95
- 20 8. The method of making shoe stiffeners which comprises impregnating porous sheet material with a stiffening substance which renders the material substantially impervious to air and moisture, and subjecting a locality spaced from the edge thereof to pressure so applied as to render that locality pervious to air and moisture. 100
- 25 9. The method of making shoe stiffeners which comprises impregnating porous sheet material with a stiffening substance which renders said material substantially impervious to air and moisture, and expelling sufficient substance from a selected locality in such manner as to render that locality pervious. 105
- 30 10. The method of making shoe stiffeners which comprises impregnating porous sheet material with a stiffening substance which renders the material substantially impervious to air and moisture, subjecting a selected locality for a predetermined interval to heat and to rolling pressure sufficient to expel some of the substance but insufficient to consolidate the sheet material, and then withdrawing the pressure and heat to permit the released fibres to pull the substance adjacent to them apart to form passages through the substance. 110
- 35 11. A shoe stiffener comprising a porous base impregnated with a stiffening substance which is impervious to air and moisture, said substance in a locality spaced from the margin of the stiffener being discontinuous sufficiently to be pervious. 115
- 40 12. A shoe stiffener comprising a porous base impregnated with a thermoplastic stiffening substance which is impervious to air and moisture, said substance in a locality spaced from the margin of the stiffener being discontinuous sufficiently to be pervious. 120
- 45 13. A shoe stiffener comprising a porous base impregnated with a stiffening substance which is impervious to air and moisture, said substance in a locality in the middle portion of the stiffener being discontinuous sufficiently to be pervious, there being located between said locality and the edge of the stiffener a narrow locality containing an excess of stiffening substance. 125
- 50 14. A shoe stiffener comprising a porous base impregnated with a stiffening substance which is impervious to air and moisture, the quantity of stiffening substance per unit volume in that portion of the stiffener which in the finished shoe will be uppermost being less than in portions adjacent to the edge of the stiffener and having a sufficient number of passages through it to render said first-named portion pervious. 130
- 55 15. A shoe stiffener comprising a porous base and a thermoplastic impregnating substance, a locality one edge of which extends substantially parallel to an edge of the stiffener containing a quantity of stiffening substance per unit volume sufficient to render that locality stiff and impervious to air and moisture, and a second locality located nearer to the center of the blank containing a lesser amount of stiffening substance per unit volume, said last-named locality being comparatively soft and resilient and pervious to air and moisture. 135
- 60 16. A shoe stiffener having a comparatively thin and flexible middle portion completely surrounded by a thicker and less flexible portion. 140
- 65 17. A shoe stiffener having a comparatively thin and flexible middle portion completely surrounded by a thicker and less flexible portion, said last-named portion being spaced from the edge of the stiffener. 145
- 70 18. A shoe stiffener having a comparatively thin and flexible middle portion completely surrounded by a thicker and less flexible portion, said last-named portion being spaced from the edge of the stiffener and said edge being at least as thin and flexible as said middle portion. 150
- 75 19. The method of making shoe stiffeners which comprises impregnating fibrous sheet material with a stiffening substance which renders the material substantially impervious to air and moisture, subjecting a selected locality for a predetermined interval to heat and pressure sufficient to expel some of the substance but insufficient to consolidate the sheet material, and then withdrawing the pressure and heat to permit the released fibres to pull the substance adjacent to them apart so as to form passages through the substance. 155
- 80 20. A shoe stiffener made from porous material impregnated with a stiffening substance, said stiffener having a middle portion of a given thickness, a rear edge the thickness of which does not exceed that of the middle portion, and two small portions of greater thickness than that of the middle portion, said two small portions being located respectively in the two angles included between the rear and the side edges of the stiffener. 160

LUCIEN PAUL MELLERIO.